



US007942983B2

(12) **United States Patent**  
**Hsu et al.**

(10) **Patent No.:** **US 7,942,983 B2**  
(45) **Date of Patent:** **May 17, 2011**

(54) **PHOSPHATING SOLUTION AND METHOD FOR CONVERSION TREATING SURFACE OF MAGNESIUM ALLOY WORKPIECE**

(75) Inventors: **Sheng-En Hsu**, Taipei Hsien (TW); **Yong Liu**, Shenzhen (CN); **Fei-Xiang Li**, Shenzhen (CN); **Zhao Jin**, Shenzhen (CN)

(73) Assignees: **Hong Fu Jin Precision Industry (ShenZhen) Co., Ltd.**, Shenzhen, Guangdong Province (CN); **Hon Hai Precision Industry Co., Ltd.**, Tu-Cheng, New Taipei (TW)

(\*) Notice: Subject to any disclaimer, the term of this patent is extended or adjusted under 35 U.S.C. 154(b) by 480 days.

(21) Appl. No.: **12/168,054**

(22) Filed: **Jul. 3, 2008**

(65) **Prior Publication Data**

US 2009/0159158 A1 Jun. 25, 2009

(30) **Foreign Application Priority Data**

Dec. 19, 2007 (CN) ..... 2007 1 0203245

(51) **Int. Cl.**

**C23C 22/57** (2006.01)  
**C23C 22/05** (2006.01)

(52) **U.S. Cl.** ..... **148/253; 148/259; 148/260; 148/262; 148/274; 148/275; 106/14.05; 106/14.12**

(58) **Field of Classification Search** ..... **148/253, 148/259, 260, 262, 274, 275; 106/14.05, 106/14.12**

See application file for complete search history.

(56) **References Cited**

**U.S. PATENT DOCUMENTS**

**2,975,082 A \*** 3/1961 Henricks ..... 148/259

\* cited by examiner

*Primary Examiner* — Roy King

*Assistant Examiner* — Lois Zheng

(74) *Attorney, Agent, or Firm* — Zhigang Ma

(57) **ABSTRACT**

An exemplary phosphating solution is used for conversion treating a surface of a magnesium alloy workpiece. The phosphating solution includes: 2.89 gram/liter to 8.67 gram/liter of phosphoric acid, 0.3 gram/liter to 1.0 gram/liter of carbamide, 0.39 gram/liter to 1.56 gram/liter of nitric acid, 6 gram/liter to 30 gram/liter of manganese dihydrogen phosphate, and 0.2 gram/liter to 0.6 gram/liter of tannin. A method for conversion treating a surface of a magnesium alloy workpiece is also provided.

**7 Claims, 4 Drawing Sheets**





FIG. 1

| Process                        | Temperature      | Time                     |
|--------------------------------|------------------|--------------------------|
| Degreasing                     | 55 °C to 60 °C   | 4 minutes to 8 minutes   |
| 1 <sup>st</sup> water cleaning | Room Temperature | 2 minutes to 19 minutes  |
| 2 <sup>nd</sup> water cleaning | Room Temperature | 2 minutes to 19 minutes  |
| 3 <sup>rd</sup> water cleaning | Room Temperature | 2 minutes to 19 minutes  |
| Acid pickling                  | 35 °C to 45 °C   | 3 minutes to 5 minutes   |
| 1 <sup>st</sup> water cleaning | Room Temperature | 2 minutes to 13 minutes  |
| 2 <sup>nd</sup> water cleaning | Room Temperature | 2 minutes to 13 minutes  |
| Alkali pickling                | 60 °C to 80 °C   | 3 minutes to 5 minutes   |
| 1 <sup>st</sup> water cleaning | 30 °C to 50 °C   | 2 minutes to 17 minutes  |
| 2 <sup>nd</sup> water cleaning | Room Temperature | 2 minutes to 17 minutes  |
| 3 <sup>rd</sup> water cleaning | Room Temperature | 2 minutes to 17 minutes  |
| Chemical converting            | 35 °C to 45 °C   | 30 seconds to 50 seconds |
| 1 <sup>st</sup> water cleaning | Room Temperature | 2 minutes to 11 minutes  |
| 2 <sup>nd</sup> water cleaning | Room Temperature | 2 minutes to 11 minutes  |
| 3 <sup>rd</sup> water cleaning | Room Temperature | 2 minutes to 11 minutes  |
| Drying                         | 110 °C to 150 °C | 30 minutes to 70 minutes |

FIG. 2

| Steps                  | Recipes<br>Solutions                 | Concentration (g/L) |      |      |
|------------------------|--------------------------------------|---------------------|------|------|
|                        |                                      | A                   | B    | C    |
| Acid pickling          | citric acid                          | 8                   | 10   | 15   |
|                        | surface active agent                 | 3                   | 3    | 4    |
| Alkali pickling        | KOH                                  | 100                 | 120  | 150  |
| Chemical<br>converting | $\text{H}_3\text{PO}_4$              | 4.34                | 5.78 | 6.5  |
|                        | $(\text{NH}_2)_2\text{CO}$           | 0.4                 | 0.5  | 0.6  |
|                        | $\text{HNO}_3$                       | 0.94                | 0.78 | 0.62 |
|                        | $\text{Mn}(\text{H}_2\text{PO}_4)_2$ | 10                  | 15   | 18   |
|                        | tannic acid                          | 0.4                 | 0.5  | 0.55 |

FIG. 3

| Samples               | Recipes  | Surface Resistance (ohm) | Corrosion Resistance | Bonding Strength |
|-----------------------|----------|--------------------------|----------------------|------------------|
| 1 <sup>st</sup> group | A column | 1.25, 1.42, 1.35         | 8, 9, 9 grade/8hours | 4B, 5B, 5B       |
| 2 <sup>nd</sup> group | B column | 0.74, 1.54, 1.65         | 9, 9, 9 grade/8hours | 5B, 5B, 5B       |
| 3 <sup>rd</sup> group | C column | 0.87, 1.34, 0.76         | 9, 9, 9 grade/8hours | 5B, 5B, 5B       |

FIG. 4

## 1

**PHOSPHATING SOLUTION AND METHOD  
FOR CONVERSION TREATING SURFACE OF  
MAGNESIUM ALLOY WORKPIECE**

**CROSS-REFERENCE TO RELATED  
APPLICATIONS**

This application is related to U.S. patent applications, applications Ser. No. 12/168,053, entitled "MAGNESIUM ALLOY ARTICLE AND METHOD FOR FABRICATING THE SAME", now abandoned; applications Ser. No. 12/168,055, entitled "ACID PICKLING SOLUTION AND METHOD FOR SURFACE TREATMENT UTILIZING THE SAME". In the co-pending applications, the inventors are Sheng-En Hsu, Yong Liu, Fei-Xiang Li and Zhao Jin. Such applications have the same assignee as the present application and have been concurrently filed herewith. The disclosures of the above identified applications are incorporated herein by reference.

**BACKGROUND**

**1. Field of the Invention**

The present invention relates phosphating solutions and methods for conversion treating surface of magnesium alloy workpieces.

**2. Discussion of the Related Art**

Magnesium is a metal that is the lightest in weight among metal materials. Magnesium alloys are composed of the magnesium and some other metals, such as aluminum and zinc. In recent years, there has been an increase in demand for magnesium alloys used as structural materials for electronic products and vehicles.

The magnesium alloy may easily react with other chemical substances such as acids, thus, a protective layer is normally needed to be formed on surfaces of magnesium alloy workpieces. A phosphating film is generally formed on an outer surface of a magnesium alloy workpiece to protect the magnesium alloy workpiece.

The phosphating film is formed by a method for conversion treating surface of the magnesium alloy workpiece. Typically, the method includes a step of chemical converting. However, the thickness of the phosphating film formed in the step of chemical converting is not easily regulated, and frequently, a corrosion resistance or a surface resistance film is not satisfactorily formed on the magnesium alloy workpiece to meet the requirements.

Therefore, a phosphating solution and method for conversion treating surface of a magnesium alloy workpiece are desired in order to overcome the above-described shortcomings.

**SUMMARY**

A phosphating solution is used for conversion treating a surface of a magnesium alloy workpiece. The phosphating solution includes: 2.89 gram/liter to 8.67 gram/liter of phosphoric acid, 0.3 gram/liter to 1.0 gram/liter of carbamide, 0.39 gram/liter to 1.56 gram/liter of nitric acid, 6 gram/liter to 30 gram/liter of manganese dihydrogen phosphate, and 0.2 gram/liter to 0.6 gram/liter of tannin.

Other advantages and novel features will become more apparent from the following detailed description of various embodiments, when taken in conjunction with the accompanying drawings.

**BRIEF DESCRIPTION OF THE DRAWINGS**

The components in the drawings are not necessarily drawn to scale, the emphasis instead being placed upon clearly illus-

## 2

trating the principles of the present phosphating solution and method for conversion treating surface of the magnesium alloy workpiece. Moreover, in the drawings, like reference numerals designate corresponding parts throughout several views.

FIG. 1 is a flowchart of a method for conversion treating surface of a magnesium alloy workpiece in accordance with an exemplary embodiment of the present invention.

FIG. 2 is a table showing temperatures and times for different steps in the method of FIG. 1.

FIG. 3 is a table showing recipes of acid pickling solutions, alkaline solutions, and phosphating solutions respectively.

FIG. 4 a table showing test results of the samples.

**DETAILED DESCRIPTION OF THE PREFERRED  
EMBODIMENTS**

Reference will now be made to the drawings to describe preferred embodiments of the present magnesium alloy workpiece, and method for making the same, in detail.

Referring to FIG. 1, a flowchart of a method for conversion treating surface of a magnesium alloy workpiece according an exemplary embodiment is shown. The method includes following steps:

Step 10, providing a magnesium alloy workpiece having a surface.

Step 20, degreasing: placing the magnesium alloy workpiece into a degreasing solution to remove oil or the like from the surface of the magnesium alloy workpiece.

Step 30, acid pickling: placing the magnesium alloy workpiece into an acid pickling solution to remove oxides and release agents from the surface of the magnesium alloy workpiece.

Step 40, alkali pickling: placing the magnesium alloy workpiece into an alkaline solution to remove black ash from the surface of the magnesium alloy workpiece.

Step 50, chemical converting: placing the magnesium alloy workpiece into a phosphating solution containing tannin to form a phosphating film on the surface of the magnesium alloy workpiece.

The method for conversion treating surface of the magnesium alloy workpiece is explained in detail below by referring to FIG. 2.

In step 20, a time period the magnesium alloy workpiece is placed in the degreasing solution is in a range from about 4 minutes to about 8 minutes, and a temperature of the degreasing solution is in range from about 55 degrees centigrade to about 65 degrees centigrade. The degreasing solution consists of sodium hydroxide (NaOH) or sodium phosphate (Na<sub>3</sub>PO<sub>4</sub>) and water (H<sub>2</sub>O). It should be pointed that, if the magnesium alloy workpiece has been treated with a sand blasting process, the oils or the like on the surface of the magnesium alloy workpiece have already been removed during the sand blasting process, the step 20 can be omitted.

In step 30, a time period the magnesium alloy workpiece is placed in the acid pickling solution is in a range from about 3 minutes to about 5 minutes, and a temperature of the acid pickling solution is in a range from about 35 degrees centigrade to about 45 degrees centigrade. The acid pickling solution consists of citric acid, surface active agent, and water (H<sub>2</sub>O). The surface active agent is water soluble and silicone free. A concentration of the citric acid is in a range from 5 gram/liter to 30 gram/liter. A concentration of the surface active agent (industrial grade) is in a range from 1.5 gram/liter to 6 gram/liter.

The citric acid may react with and remove the oxides and release agent from the surface of the magnesium alloy work-

piece. The oxides can be magnesia ( $\text{MgO}$ ), alumina ( $\text{Al}_2\text{O}_3$ ), and zinc oxide ( $\text{ZnO}$ ). The release agents include a resin represented by a formula:  $(\text{CH}_2)_m-\text{CH}(\text{Si})_n-\text{COOR}$ , wherein, R represents a functional group such as methyl. The citric acid may also prevent the black ash (the main gradient of the black ash is Al and Zn) from forming on the surface of the magnesium alloy workpiece to a certain extent. A concentration of the citric acid is in a range from 8 gram/liter to 15 gram/liter. When the magnesium alloy workpiece is placed into the acid pickling solution, the following chemical reactions may occur:



The surface active agent may be used as a buffer, so as to prevent excessive corrosion to the magnesium alloy workpiece. The surface active agent includes a hydrophilic group, such as a hydroxyl. The surface active agent can be a polyalcohol, such as poly ethylene glycol, glycerol, neopentyl glycol, sucrose, dextrose, or sorbitol. A concentration of the surface active agent is in a range from 3 gram/liter to 4 gram/liter.

In step 40, a time period of the magnesium alloy workpiece is placed in the alkaline solution is in a range from about 3 minutes to about 5 minutes, and a temperature of the alkaline solution is in a range from about 60 degrees centigrade to about 80 degrees centigrade. A solute of the alkaline solution can be potassium hydroxide (KOH) or sodium hydroxide (NaOH).

The alkaline solution is mainly used to react with and remove the black ash from the surface of the magnesium alloy workpiece such that a base of the magnesium alloy workpiece is exposed. When the solute is KOH (industrial grade), a concentration of the KOH is in a range from 60 gram/liter to 180 gram/liter. Preferably, a concentration of the KOH is in the range from 100 gram/liter to 150 gram/liter. When the magnesium alloy workpiece is placed into the alkaline solution, the following chemical reactions may occur:



In step 50, a time period the magnesium alloy workpiece is placed in the phosphating solution is in a range from about 30 seconds to about 50 seconds, and a temperature of the phosphating solution is in a range from about 35 degrees centigrade to about 45 degrees centigrade. The thickness of the phosphating film formed on the surface of the workpiece can be in a range from 5 microns to 30 microns. A surface resistance of the phosphating film formed on the magnesium alloy workpiece is less than 2 ohms. The phosphating solution can include 2.89 gram/liter to 8.67 gram/liter of phosphoric acid ( $\text{H}_3\text{PO}_4$ ) (industrial grade), 0.3 gram/liter to 1.0 gram/liter of carbamide ( $(\text{NH}_2)_2\text{CO}$ ) (Analytical Reagent Grade), 0.39 gram/liter to 1.56 gram/liter of nitric acid ( $\text{HNO}_3$ ) (industrial grade), 2 gram/liter to 30 gram/liter of manganese dihydrogen phosphate ( $\text{Mn}(\text{H}_2\text{PO}_4)_2$ ) (industrial grade), and 0.2 gram/liter to 0.6 gram/liter of tannin ( $\text{C}_{76}\text{H}_{52}\text{O}_{46}$ ) (Analytical Reagent Grade).

The  $\text{H}_3\text{PO}_4$  is used to provide  $\text{PO}_4^{3-}$  ions. To further regulate a thickness of the phosphating film formed on the surface of the workpiece, the concentration of the  $\text{H}_3\text{PO}_4$  is, preferably, in the range from 4.34 gram/liter to 6.5 gram/liter.

5 The  $(\text{NH}_2)_2\text{CO}$  is used to make the phosphating film uniformly. To prevent the phosphating film from developing/forming too slowly, the concentration of the  $(\text{NH}_2)_2\text{CO}$  is, preferably, in the range from 0.4 gram/liter to 0.6 gram/liter.

The  $\text{HNO}_3$  is used to provide  $\text{H}^+$  ions to adjust a PH value 10 of the phosphating solution to be in a range from about 6.5 to about 9.5. Preferably, the concentration of the  $\text{HNO}_3$  is in the range from 0.62 gram/liter to 0.94 gram/liter.

15 The  $\text{Mn}(\text{H}_2\text{PO}_4)_2$  is used to provides  $\text{Mn}^{2+}$ ,  $\text{PO}_4^{3-}$ , and  $\text{H}^+$  ions. To further regulate to form a more uniform thickness of the phosphating film on the surface of the workpiece, the concentration of the  $\text{Mn}(\text{H}_2\text{PO}_4)_2$  is, preferably, in the range from 10 gram/liter to 18 gram/liter.

20 The tannin is used to improve an bonding strength between the phosphating film and a painting layer coated on the phosphating film. Preferably, the concentration of the tannin is in the range from 0.4 gram/liter to 0.55 gram/liter.

25 The phosphating film mainly consists of composite phosphates including  $\text{Mg}_3(\text{PO}_4)_2$ ,  $\text{Mn}_3(\text{PO}_4)_2$ , and so on. When the magnesium alloy workpiece is placed into the phosphating solution, the following chemical reactions may occur;



30 The formula of the composite phosphate can be:



35 It can be understood that, the method can further include a water cleaning step after the step 20, step 30, step 40, and step 50 respectively. In addition, the method may include a drying process after the step 50. The magnesium alloy workpiece can be dried at a temperature in a range from about 110 degrees centigrade to about 150 degrees centigrade for a time period 40 in a range from about 30 minutes to about 70 minutes.

45 Examples of methods for conversion treating surface of the magnesium alloy workpieces are described as follows.

45 Three groups (1<sup>st</sup> group, 2<sup>nd</sup> group, and 3<sup>rd</sup> group, each including three magnesium alloy workpieces) of magnesium alloy workpieces are provided. A material of each of the magnesium alloy workpiece is AZ91D. The three groups of magnesium alloy workpieces are treated with the processes shown in FIG. 2 correspondingly, thereby yielding three 50 groups of samples of magnesium alloy products. As shown in FIG. 3, Recipes (A column, B column, and C column) of acid pickling solutions, alkline treatment solutions, and phosphating solutions are used during the corresponding processes of the three sample groups (1<sup>st</sup> group, 2<sup>nd</sup> group, and 3<sup>rd</sup> group) 55 of magnesium alloy workpiece.

55 Corrosion resistance of the samples are evaluated by a salt spray tester. A salt spray test solution used in the salt spray tester includes 5% of sodium chloride (NaCl). Surface resistances of the samples of the magnesium alloy products are evaluated by using micro-ohmmeter. Bonding strength of the samples of the magnesium alloy products is evaluated by cross-cut test after an outer coating is formed on the phosphating film. Referring to FIG. 4, a test result of the samples is shown. Corrosion resistance of the samples of the magnesium alloy products are all above grade 8, the surface resistances of samples of the magnesium alloy products are all less than 2 ohms, and bonding strength of the samples of the

magnesium alloy products are all above 3B grade. Therefore, the magnesium alloy products all have good corrosion resistance, relatively high bonding strength, and low surface resistance. It is understood that, if the magnesium alloy products are used to make a portable electronic devices, the portable electronic devices may have a good electromagnetic interference shielding efficiency.

Finally, while various embodiments have been described and illustrated, the invention is not to be construed as being limited thereto. Various modifications can be made to the embodiments by those skilled in the art without departing from the true spirit and scope of the invention as defined by the appended claims.

What is claimed is:

1. A phosphating solution for conversion treating a surface of a magnesium alloy workpiece, the phosphating solution comprising: 2.89 gram/liter to 8.67 gram/liter of phosphoric acid, 0.3 gram/liter to 1.0 gram/liter of carbamide, 0.39 gram/liter to 1.56 gram/liter of nitric acid, 6 gram/liter to 30 gram/liter of manganese dihydrogen phosphate, and 0.2 gram/liter to 0.6 gram/liter of tannin.

2. The phosphating solution for conversion treating a surface of a magnesium alloy workpiece as claimed in claim 1, wherein the phosphoric acid is in the range from 4.34 gram/liter to 6.50 gram/liter.

3. The phosphating solution for conversion treating a surface of a magnesium alloy workpiece as claimed in claim 1, wherein the carbamide is in the range from 0.4 gram/liter to 0.6 gram/liter.

4. The phosphating solution for conversion treating a surface of a magnesium alloy workpiece as claimed in claim 1, wherein the nitric acid is in the range from 0.62 gram/liter to 0.94 gram/liter.

5. The phosphating solution for conversion treating a surface of a magnesium alloy workpiece as claimed in claim 1, wherein the manganese dihydrogen phosphate is in the range from 10 gram/liter to 18 gram/liter.

10 6. The phosphating solution for conversion treating a surface of a magnesium alloy workpiece as claimed in claim 1, wherein the tannin is in the range from 0.4 gram/liter to 0.55 gram/liter.

7. The phosphating solution for conversion treating a surface of a magnesium alloy workpiece as claimed in claim 1, 20 wherein a PH value of the phosphating solution is in the range from about 6.5 to about 9.5.

\* \* \* \* \*